

# UNITED STATES PATENT OFFICE.

ANTHONY MAURICE KOHLER, OF BRIXTON, LONDON, ENGLAND.

## ELECTROCHEMICAL PROCESS FOR CLEANING AND POLISHING SILVER PLATE AND THE LIKE.

983,727.

Specification of Letters Patent.

Patented Feb. 7, 1911.

No Drawing.

Application filed July 6, 1909. Serial No. 506,166.

To all whom it may concern:

Be it known that I, ANTHONY MAURICE KOHLER, a citizen of the Republic of Switzerland, and resident of 21 St. Ann's road, 5 Brixton, in the county of London, England, have invented certain new and useful Improvements in Electrochemical Processes for Cleaning and Polishing Silver Plate and the Like, (for which I have obtained a patent 10 in Great Britain, No. 15,962, bearing date July 27, 1908,) of which the following is a specification.

This invention relates to a process whereby silver plate and the like may be cleaned 15 and polished by immersing the article under treatment in an alkaline solution in the presence of aluminium or any alloy containing it in any proportion.

According to the present invention this 20 cleaning and polishing solution may be made by dissolving any alkali or mixture of alkalis in water, and any suitable salt, powder or dye in any form may be added to the solution to give it color or increase its chemical action. The solution may be used hot or 25 cold at any suitable temperature, and it may be contained in a vessel of any suitable shape, made of silver, china, silver plate or any suitable material. The aluminium or the 30 alloy containing it may be partly or fully immersed in the solution and it may be in any suitable form or shape and in any quantity.

The chemical action taking place in accordance with the process forming the subject of my invention, when soda and aluminium are used, is as follows:—



40 but use can be made of any alkaline solution or any aluminium alloy.

When the article or articles are immersed in the solution and touch or are otherwise connected with the aluminium or alloy 45 thereof employed, a chemical action takes place, causing hydrogen to be liberated by decomposition, and this combining with the metallic oxides that really forms the "tarnish" on the surface of the article to be polished, thus forms water, leaving the surface as bright as it originally was before it was oxidized or tarnished. The separation of the hydrogen from the alkaline liquid causes a certain amount of the aluminium hydroxid 55 or alloy thereof to be dissolved, which again

forms aluminium hydroxid  $\text{Al}(\text{OH})_3$ , in addition to the respective hydroxides (if an alloy is employed, and depending on the kind of alloy) which would in some cases be reduced to  $\text{Al}(\text{OH})_2$  due to the presence of 60 aluminium, or otherwise accomplish the same result as the aluminium hydroxid, *i. e.* in producing various sets of compounds or salts according to the composition of the alloy when such is employed, thus forming a 65 slight white film upon the surface of the article to be polished which may be removed by rubbing and leave said surface perfectly bright and clean.

Although I have mentioned  $\text{NaOH}$  as a 70 preferable alkaline solution, I may in some cases use a solution of the salts of other alkaline metals, and the percentage of alkali in the solution depends on the quantity and 75 quality of the articles to be cleaned and polished, and the proportions would therefore vary, and in the employment of an alloy of aluminium the percentage of aluminium in such alloy would also depend on the quantity and quality of the articles to be cleaned 80 and polished, and these proportions would also vary.

An example of an alloy to be used in place of aluminium is as follows:

|                               |            |
|-------------------------------|------------|
| Aluminium                     | 80 parts.  |
| Barium                        | 10 parts.  |
| Calcium                       | 8 parts.   |
| Sodium                        | 1 part.    |
| Silicium and other impurities | 1 part.    |
|                               | 90         |
|                               | 100 parts. |

This alloy may be partly or fully immersed in the solution and it may be in any suitable form or shape and in any quantity. 95 When such an alloy as above is employed the chemical action taking place in accordance with the process forming the subject of this invention, when soda is the alkali, is such that some of the alloy constituents, as 100 for instance aluminium, are attacked by the alkaline solution, forming its respective salt, thus:—



Said salt or compound may take part in the polishing process straightway, or in some cases is decomposed, producing compounds such as aluminium hydroxid, depending on 110 the alloy or alkaline solution used.

Other of the alloy constituents such as sodium may form their respective hydroxid straightway, thus:—



5 If the articles to be cleaned are greasy or very much soiled, they may be immersed in a heated solution of  $\text{NaCO}_3$  before placing in the solution for polishing hereinbefore described.

Having now described my invention, what I claim as new and desire to secure by Letters Patent of the United States is:—

10 A process of cleaning and polishing plated

articles and the like, which consists in immersing in a receptacle containing an aluminium salt solution, aluminium and the article to be cleaned, hydrogen thereby being liberated and combined with the oxid on the article to produce water, and afterward drying the article.

20 In testimony whereof I have affixed my signature in presence of two witnesses.

ANTHONY MAURICE KOHLER.

Witnesses:

BENJN. THOS. KING,  
ROBT. HUNTER.